# EUROPEAN PATENT SPECIFICATION

(11) **EP 3 271 503 B1**
(45) Date of publication and mention of the grant of the patent: **21.11.2018**
(21) Application number: 16722365.0
(22) Date of filing: 18.03.2016
(51) Int. Cl.: D02G 3/28

(54) **METHOD FOR MANUFACTURING A SILK-BASED FABRIC AND USE OF THE FABRIC**
VERFAHREN ZUR HERSTELLUNG EINES STOFFS AUF BASIS VON SEIDE UND VERWENDUNG DES STOFFS
PROCÉDÉ DE FABRICATION D'UN TISSU À BASE DE SOIE ET UTILISATION DE CE TISSU

(30) Priority: 20.03.2015 IT UB20150431
(43) Date of publication of application: 24.01.2018
(73) Proprietor: Lanificio Ermenegildo Zegna & Figli S.p.A., 13835 Trivero (Biella) (IT)
(72) Inventor: FERRARIS, Augusto, 13835 Trivero (Biella) (IT)
(74) Representative: De Filippis, Sara
(86) International application number: PCT/IB2016/051530
(87) International publication number: WO 2016/151448

(56) References cited:
- EP-A1- 2 426 241
- CN-A- 104 108 327
- KR-B1- 100 914 335

## Description

The present invention relates to a method for manufacturing a silk-based fabric.

More specifically, the invention relates to a method for manufacturing a silk-based fabric for use as a covering in a passenger compartment of a motor vehicle, in particular for seats and the like, of the type comprising the steps of:
manufacturing a twisted silk yarn having predetermined characteristics, and
manufacturing an orthogonal woven fabric with warp and weft threads manufactured using said twisted yarn.

A method of this type is described in the aforementioned Italian patent application TO2014A000474 in the name of the same Applicant.

According to the method described in this prior patent application a silk-based twisted yarn is made from strips of discontinuous silk fibres which are subjected to fibre opening and then to a carding process.

KR-B-100 914 333 discloses a method for manufacturing a silk-based fabric comprising the steps of manufacturing a twisted silk yarn having predetermined features and knitting said twisted yarn e.g. in a pullover.

EP-A-2 426 241 discloses the purification of silk to eliminate immunogenic components, such as sericin, and the use of the purified silk to form tissue-supporting prosthetic devices for implantation.

CN-A-104 108 327 discloses a seat cushion of an automobile comprising a head pad, a back pad and a hip pad.

One object of the present invention is to propose an improved method which allows the manufacture of silk-based fabrics which can be used in the furnishing sector and in particular for furnishing the passenger compartments of motor vehicles, for covering seats,

bench seats and the like.

The fabrics used for these applications must have, in addition to other characteristics, also a high wear-resistance, which per se cannot be easily ensured when silk-based yarns are used, as well as low emissions for limiting the generation of so-called fogging effects, for example on the glass surfaces of a motor vehicle.

The aforementioned object and other objects are achieved according to the invention with a method of the type defined above, characterized primarily in that:
* the manufacture of the aforementioned twisted yarn comprises the steps of:
   - providing first and second single-thread yarns of raw silk having a metric count equal to or greater than 80 and Z-type twist equal to or greater than 600 turns/linear metre;
   - doubling and twining said first and second yarns, one with the other, so as to provide doubled and twined yarns having an S-type twist equal to or greater than 350 turns/linear metre;
   - skein-dyeing and subsequently winding-off said doubled and twined yarns; and
   - preparing said twisted yarn by plying and twisting a plurality of said doubled and twined yarns;
   and in that
* the manufacture of the aforementioned fabric comprises the steps of:
   - preparing a warp with said twisted yarn, with a thread density of more than 20 threads per centimetre, without applying to the warp threads any oils or waxes, and
   - weaving the warp with weft threads, with a density greater than 18 weft threads per centimetre, without applying to the weft threads any oils or waxes.

The present invention also relates to particular uses of fabrics made with a method of the type defined above.

Further characteristic features and advantages of the invention will become clear from the following description provided purely by way of a non-limiting example.

For the manufacture of a silk-based fabric which can be used in particular for covering seats and the like, such as single seats or bench seats in motor vehicles, the method according to the present invention envisages initially the manufacture of a twisted silk yarn with predetermined characteristics.

In particular, the manufacture of this twisted yarn comprises the operation of providing first and second single-thread yarns of raw silk having a metric count Nm (km of yarn per kilogram) equal to or greater than 80 and Z-type twist equal to or greater than 600 turns/linear metre.

Preferably, said first and second silk yarns have a metric count Nm comprised between 80 and 120 and a Z-type twist comprised between 600 and 800 turns/linear metre.

These first and second silk yarns are then doubled and twined together so as to provide yarns having an S-type twist comprised between 350 and 600 turns/linear metre.

Dyeing of these doubled and twined yarns is then performed. These yarns are in particular skein-dyed and then wound off using preferably an off-reeling machine with automatic knotting using thermo-splicer technology.

After dyeing, using these doubled and twined yarns a twisted yarn is prepared by plying and twisting three threads of said doubled and twined yarns, with an S-type twist comprised between 300 and 500 turns/linear metre.

Thereafter, depending on whether an orthogonal fabric or weft and warp fabric is to be made, a warp is prepared using the twisted yarn described above.

The warp is prepared with a thread density greater than 20 threads per centimetre.

In order to limit drastically the occurrence, during use, of fogging, the application of any oils, waxes or the like to the warp threads must be avoided.

The orthogonal fabric is then prepared in a loom set up with the warp prepared as described above, inserting weft yarns likewise obtained from the aforementioned twisted yarn, with a density greater than 18 weft threads per centimetre.

In order to limit drastically the occurrence, during use, of fogging, the application of any oils, waxes or the like to the weft threads must be avoided.

Optimum results have been obtained with a warp having a thread density comprised between 20 and 30 threads per centimetre and with a weft density likewise comprised between 20 and 30 threads per centimetre.

Conveniently, the fabric is manufactured with a twill weave, in particular a Batavia or Casimir twill weave, which results in the formation of a fabric with a design for example of the herringbone type.

The orthogonal fabric thus manufactured is then subjected, in sequence, to operations of washing, drying, singeing in a gassing machine, washing and drying in a stenter machine. The fabric may then be subjected to operations of anti-UV treatment and drying in a stenter machine.

Conveniently, the fabric may then be subjected to wear-prevention treatment, by means of foulard application of resins or the like, followed by drying in a stenter machine and decatizing.

The use of the twined doubled yarn as described above for the manufacture of the fabric has proved to be a decisive measure for the purposes of obtaining a fabric characterized by a very high wear resistance. This fabric is therefore suitable for use in "heavy duty" applications, in particular for covering seats or bench seats.

The scope of the present invention therefore also embraces the use of a fabric manufactured with the method defined above, for covering seats and the like, and in particular single seats or bench seats of motor vehicles.

In a motor vehicle, in addition to the seats, other parts may also be advantageously provided with a fabric covering or the like.

This is the case for example with wall coverings, as in the case of door panels or the roof of the passenger compartment.

These wall linings may be conveniently manufactured with a knitted fabric, obtained using a twisted silk yarn obtained by twisting, after dyeing, a plurality (preferably two) doubled and twined yarns having an S-type twist greater than or equal to 350 turns/linear metre and preferably comprised between 350 and 600 turns/linear metre, each of said doubled and twined yarns being obtained by doubling and twisting a first and a second single-thread yarn of raw silk each having a metric count Nm equal to or greater than 80 and preferably comprised between 80 and 120, and a Z-type twist, equal to or greater than 600 turns/linear metre and preferably comprised between 600 and 800 turns/linear metre.

Said knitted fabric is conveniently a Jersey-type yarn made using a circular disk machine of the conventional type.

The fabric thus manufactured is then subjected to finishing and in particular flattening operations in a stenter machine and selvedge bonding, washing, singeing in a gassing machine, washing, anti-UV treatment, drying in a stenter machine, wear-prevention treatment in a bath and decatizing.

Obviously, without altering the principle of the invention, the embodiments and the constructional details may be greatly varied with respect to that described and illustrated purely by way of a non-limiting example, without thereby departing from the scope of the invention as defined in the accompanying claims.

## Claims

1. Method for manufacturing a silk-based fabric for use as a covering in a passenger compartment of a motor vehicle, in particular for seats, comprising the steps of:
manufacturing a twisted silk yarn having predetermined characteristics, and
manufacturing an orthogonal woven fabric with warp and weft threads manufactured using said twisted yarn;
the method being **characterized in that**
* the manufacture of said twisted yarn comprises the steps of:
- providing first and second single-thread yarns of raw silk having a metric count (Nm) equal to or greater than 80 and a Z-type twist equal to or greater than 600 turns/linear metre;
- doubling and twining said first and second yarns, one with the other, so as to provide doubled and twined yarns having an S-type twist equal to or greater than 350 turns/linear metre;
- skein-dyeing said doubled and twined yarns and subsequently winding-off said skein; and
- preparing said twisted yarn by plying and twisting a plurality of said doubled and twined yarns - preferably three of said doubled and twined yarns - with an S-type twist comprised between 300 and 500 turns/linear metre,
and **in that**
* the manufacture of said fabric comprises the steps of:
- preparing a warp with said twisted yarn, with a thread density of more than 20 threads/centimetre, without applying to the warp threads any oils or waxes, and
- weaving the warp with weft threads, with a density greater than 18 weft threads/centimetre, without applying to the weft threads any oils or waxes.

2. Method according to Claim 1, wherein said first and second silk yarns have a metric count comprised between 80 and 120 and a Z-type twist comprised between 600 and 800 turns/linear metre.

3. Method according to Claim 1 or Claim 2, wherein said first and second yarns are doubled and twined with an S-type twist comprised between 350 and 600 turns/linear metre.

4. Method according to any one of the preceding claims, wherein the density of the warp threads is comprised between 20 and 30 threads/centimetre, and the weft density is likewise comprised between 20 and 30 threads/cm.

5. Method according to any one of the preceding claims, wherein the fabric is manufactured with a twill weave, in particular a Batavia or Casimir twill weave.

6. Method according to any one of the preceding claims, wherein the fabric is subjected, in sequence, to operations of washing, drying, singeing in a gassing machine, washing and drying in a stenter machine.

7. Method according to Claim 6, wherein the fabric is further subjected to operations of anti-UV treatment and drying in a stenter machine.

8. Method according to Claim 6 or Claim 7, wherein the fabric is further subjected to wear-prevention treatment, drying in a stenter machine and decatizing.

9. Use of a fabric manufactured using the method according to one or more of the preceding claims for covering seats and the like, in particular single seats or bench seats of motor vehicles.

10. Seat, particularly for motor vehicles, covered at least in part by a fabric manufactured using a method according to any one of Claims 1 to 8.

11. Motor vehicle comprising at least one seat according to Claim 10.

12. Motor vehicle, according to Claim 11, comprising further at least one wall covering made of a knitted fabric manufactured using a silk-based yarn.

13. Motor vehicle according to Claim 12, wherein said knitted fabric is manufactured using a twisted silk yarn obtained by twisting, after dyeing, a plurality of doubled and twined silk yarns with an S-type twist greater than or equal to 350 turns/linear metre, each of said doubled and twined silk yarns being obtained by doubling and twining a first and a second single-thread yarn of raw silk, each having a metric count equal to or greater than 80 and a Z-type twist equal to or greater than 600 turns/linear metre.

14. Motor vehicle according to Claim 13, wherein said knitted fabric is a Jersey-type fabric.

15. Method for manufacturing a seat, particularly for motor vehicles, **characterized in that** the seat is covered at least in part by a fabric manufactured using a method according to any one of Claims 1 to 8.

## Patentansprüche

1. Verfahren zum Herstellen eines Stoffs auf Seidenbasis zur Verwendung als eine Abdeckung in einem Fahrgastraum eines Kraftfahrzeugs, insbesondere für Sitze, umfassend die Schritte von:
Herstellen eines verdrillten Seidengarns mit vorbestimmten Eigenschaften und
Herstellen eines orthogonal gewebten Stoffs mit Kett- und Schussfäden, die unter Verwendung des verdrillten Garns hergestellt wurden;
wobei das Verfahren **dadurch gekennzeichnet ist, dass**
* die Herstellung des verdrillten Garns die Schritte umfasst von:
- Bereitstellen eines ersten und eines zweiten eingängigen Garns aus Rohseide, das eine metrische Nummer (Nm) gleich oder größer als 80 und eine Z-Typ-Verdrillung gleich oder größer als 600 Windungen/laufendem Meter aufweist;
- Dublieren und Zwirnen des ersten und des zweiten Garns miteinander, um ein dubliertes und verzwirntes Garn bereitzustellen, das eine S-Typ-Verdrillung gleich oder größer als 350 Windungen/laufendem Meter aufweist;
- Docken-Färben des dublierten und verzwirnten Garns und nachfolgendes Abwickeln der Docke; und
- Erstellen des verdrillten Garns durch Doppeln und Verdrillen einer Vielzahl von den dublierten und verzwirnten Garnen - vorzugsweise drei von den dublierten und verzwirnten Garnen - mit einer S-Typ-Verdrillung, die zwischen 300 und 500 Windungen/laufendem Meter umfasst,
and dadurch, dass
* die Herstellung des Stoffs die Schritte umfasst von:
- Erstellen einer Kette mit dem verdrillten Garn mit einer Fadendichte von mehr als 20 Fäden/Zentimeter, ohne dass irgendwelche Öle oder Wachse auf die Kettfäden aufgebracht werden, und
- Weben der Kette mit Schussfäden mit einer Dichte größer als 18 Schussfäden/Zentimeter, ohne dass irgendwelche Öle oder Wachse auf die Schussfäden aufgebracht werden.

2. Verfahren nach Anspruch 1, wobei das erste und das zweite Seidengarn eine metrische Nummer zwischen 80 und 120 und eine Z-Typ-Verdrillung zwischen 600 und 800 Windungen/laufendem Meter aufweist.

3. Verfahren nach Anspruch 1 oder Anspruch 2, wobei das erste und das zweite Garn mit einer S-Typ-Verdrillung, die zwischen 350 und 600 Windungen/laufendem Meter umfasst, dubliert und verzwirnt werden.

4. Verfahren nach einem der vorstehenden Ansprüche, wobei die Dichte der Kettfäden zwischen 20 und 30 Fäden/Zentimeter beträgt und wobei die Schussdichte ebenfalls zwischen 20 und 30 Fäden/Zentimeter beträgt.

5. Verfahren nach einem der vorstehenden Ansprüche, wobei der Stoff mit einer Körperbindung, insbesondere einer Batavia- oder Casimir-Köperbindung, hergestellt wird.

6. Verfahren nach einem der vorstehenden Ansprüche, wobei der Stoff der Reihe nach Vorgängen des Waschens, des Trocknens, des Sengens in einer Begasungsmaschine, des Waschens und des Trocknens in einer Spannmaschine unterworfen wird.

7. Verfahren nach Anspruch 6, wobei der Stoff weiter Vorgängen einer UV-Schutzbehandlung und des Trocknens in einer Spannmaschine unterworfen wird.

8. Verfahren nach Anspruch 6 oder Anspruch 7, wobei der Stoff weiter einer Verschleißschutzbehandlung, einem Trocknen in einer Spannmaschine und einem Dekatieren unterworfen wird.

9. Verwenden eines Stoffs, der unter Verwendung des Verfahrens nach einem oder mehreren der vorstehenden Ansprüche hergestellt worden ist, zum Abdecken von Sitzen und dergleichen, insbesondere einzelnen Sitzen oder Sitzbänken von Kraftfahrzeugen.

10. Sitz, insbesondere für Kraftfahrzeuge, der zumindest teilweise durch einen Stoff abgedeckt ist, der unter Verwendung eines Verfahrens nach einem der Ansprüche 1 bis 8 hergestellt worden ist.

11. Kraftfahrzeug, umfassend zumindest einen Sitz nach Anspruch 10.

12. Kraftfahrzeug nach Anspruch 11, weiter umfassend zumindest eine Wandabdeckung, die aus einem gestrickten Stoff, der unter Verwendung eines Garns auf Seidenbasis hergestellt worden ist, gefertigt ist.

13. Kraftfahrzeug nach Anspruch 12, wobei der gestrickte Stoff unter Verwendung eines verdrillten Seidengarns hergestellt ist, das erhalten wird durch Verdrillen, nach einem Färben, einer Vielzahl von dublierten und verzwirnten Seidengarnen mit einer S-Typ-Verdrillung gleich oder größer als 350 Windungen/laufendem Meter, wobei jedes der dublierten und verzwirnten Seidengarne durch Dublieren und Zwirnen eines ersten und eines zweiten eingängigen Garns aus Rohseide erhalten wird, wobei jedes eine metrische Nummer gleich oder größer als 80 und eine Z-Typ-Verdrillung gleich oder größer als 600 Windungen/laufendem Meter aufweist.

14. Kraftfahrzeug nach Anspruch 13, wobei der gestrickte Stoff ein Jersey-artiger Stoff ist.

15. Verfahren zum Herstellen eines Sitzes, insbesondere für Kraftfahrzeuge, **dadurch gekennzeichnet, dass** der Sitz zumindest teilweise durch einen Stoff abgedeckt wird, der unter Verwendung eines Verfahrens nach einem der Ansprüche 1 bis 8 hergestellt worden ist.

## Revendications

1. Procédé de fabrication d'un tissu à base de soie pour une utilisation en tant que revêtement dans un habitacle d'un véhicule motorisé, en particulier pour des sièges, comprenant les étapes de :
fabrication d'un fil de soie retors ayant des caractéristiques prédéterminées, et
fabrication d'un tissu tissé orthogonal avec des fils de chaîne et de trame fabriqués en utilisant ledit fil retors ;
le procédé étant **caractérisé en ce que**
* la fabrication dudit fil retors comprend les étapes de :
- fourniture de premier et second fils à un seul fil en soie brute ayant un numéro métrique (Nm) supérieur ou égal à 80 et une torsion Z supérieure ou égale à 600 tours/mètre linéaire ;
- doublage et tressage desdits premier et second fils, l'un avec l'autre, de façon à fournir des fils doublés et tressés ayant une torsion S supérieure ou égale à 350 tours/mètre linéaire ;
- teinture en écheveaux desdits fils doublés et tressés et ensuite déroulement desdits écheveaux ; et
- préparation dudit fil retors par retordement et torsion d'une pluralité desdits fils doublés et tressés - de préférence trois desdits fils doublés et tressés - avec une torsion S comprise entre 300 et 500 tours/mètre linéaire,
et **en ce que**
* la fabrication dudit tissu comprend les étapes de :
- préparation d'une chaîne avec ledit fil retors, avec une densité de fil de plus de 20 fils/centimètre, sans application sur les fils de chaîne d'huiles ou de cires quelconques, et
- tissage de la chaîne avec des fils de trame, avec une densité supérieure à 18 fils de trame/centimètre, sans application sur les fils de trame d'huiles ou de cires quelconques.

2. Procédé selon la revendication 1, dans lequel lesdits premier et second fils de soie ont un numéro métrique compris entre 80 et 120 et une torsion Z comprise entre 600 et 800 tours/mètre linéaire.

3. Procédé selon la revendication 1 ou la revendication 2, dans lequel lesdits premier et second fils sont doublés et tressés avec une torsion S comprise entre 350 et 600 tours/mètre linéaire.

4. Procédé selon l'une quelconque des revendications précédentes, dans lequel la densité des fils de chaîne est comprise entre 20 et 30 fils/centimètre, et la densité de la trame est de même comprise entre 20 et 30 fils/cm.

5. Procédé selon l'une quelconque des revendications précédentes, dans lequel le tissu est fabriqué avec une armure croisée, en particulier une armure croisée Batavia ou Casimir.

6. Procédé selon l'une quelconque des revendications précédentes, dans lequel le tissu est soumis, successivement, à des opérations de lavage, séchage, flambage dans une machine de gazage, lavage et séchage dans une machine élargisseuse.

7. Procédé selon la revendication 6, dans lequel le tissu est en outre soumis à des opérations de traitement anti-UV et de séchage dans une machine élargisseuse.

8. Procédé selon la revendication 6 ou la revendication 7, dans lequel le tissu est en outre soumis à un traitement de prévention de l'usure, de séchage dans une machine élargisseuse et de décatissage.

9. Utilisation d'un tissu fabriqué en utilisant le procédé selon une ou plusieurs des revendications précédentes pour le revêtement de sièges et autres, en particulier de sièges individuels ou de banquettes de véhicules motorisés.

10. Siège, en particulier pour des véhicules motorisés, revêtu au moins en partie d'un tissu fabriqué en utilisant un procédé selon l'une quelconque des revendications 1 à 8.

11. Véhicule motorisé comprenant au moins un siège selon la revendication 10.

12. Véhicule motorisé, selon la revendication 11, comprenant en outre au moins un revêtement de paroi fait d'un tissu tricoté fabriqué en utilisant un fil à base de soie.

13. Véhicule motorisé selon la revendication 12, dans lequel ledit tissu tricoté est fabriqué en utilisant un fil de soie retors obtenu par torsion, après teinture, d'une pluralité de fils de soie doublés et tressés avec une torsion S supérieure ou égale à 350 tours/mètre linéaire, chacun desdits fils de soie doublés et tressés étant obtenu par doublage et tressage d'un premier et d'un second fil à un seul fil en soie brute, chacun ayant un numéro métrique supérieur ou égal à 80 et une torsion Z supérieure ou égale à 600 tours/mètre linéaire.

14. Véhicule motorisé selon la revendication 13, dans lequel ledit tissu tricoté est un tissu de type Jersey.

15. Procédé de fabrication d'un siège, en particulier pour véhicules motorisés, **caractérisé en ce que** le siège est revêtu au moins en partie d'un tissu fabriqué en utilisant un procédé selon l'une quelconque des revendications 1 à 8.
